

Patented July 14, 1936

2,047,355

# UNITED STATES PATENT OFFICE

2,047,355

## MOTOR FUEL

Edmund G. Borden, Little Neck, N. Y., assignor to  
Gasoline Antioxidant Company, Wilmington,  
Del., a corporation of Delaware

No Drawing. Application July 26, 1933,  
Serial No. 682,269

7 Claims. (Cl. 44—9)

This invention relates to the stabilization of motor fuels and more particularly to motor fuels of the gasoline type wherein the gasoline contains hydrocarbons having gum-forming constituents.

The gasolines now being manufactured from petroleum and coal tar oils often contain unsaturated hydrocarbons which are gum-forming constituents. The modern cracking processes which decompose oils under heat and pressure tend to form unsaturated hydrocarbons, such as the olefines, diolefines, naphthenes and acetylenes. These unsaturated hydrocarbons often contain and are themselves products which are easily oxidizable and which are gum-forming constituents. The gummy material appears to be formed by oxidation whereby a flocculent sticky precipitate forms in the gasoline, the formation of this precipitate often being accelerated by sunlight. Usually when gummy materials form in the gasoline the color of the gasoline is changed. The formation of gum tends to affect both the color of the gasoline and a clouding or precipitation of a gummy product in the gasoline. The formation and removal of gum-forming constituents tends to affect the boiling range of the gasoline and also the octane rating of the gasoline.

One object of the invention is to provide a method of stabilizing the gasoline whereby gum-forming constituents will not precipitate.

Another object of the invention is to stabilize the color of the gasoline so that its color will remain substantially unchanged when standing for long periods of time.

Another object of the invention is to stabilize the octane rating of the gasoline so that its octane rating will become substantially fixed and whereby the hydrocarbon content of the gasoline which gives it the desired octane rating may be preserved.

Another object of the invention is to provide a method of treating gasoline to inhibit the formation of gum in the gasoline.

Heretofore poly-hydroxy-benzenes such as pyrogallol, catechol and resorcinol have been used as gasoline stabilizers. These compounds while good gasoline stabilizers, particularly catechol and pyrogallol, have objections which are quite effectively overcome by the present invention. For example, pyrogallol and catechol, are quite soluble in water and sparingly soluble

in gasoline. Practically all gasoline is associated with water in its transportation and storage and this objection has materially reduced the amount of pyrogallol and pyrocatechol used in stabilizing gasoline. Due to these facts it often happens that if a gasoline is stabilized with pyrogallol and then brought into contact with water, the pyrogallol is practically all removed from the gasoline and the stabilizing effect of pyrogallol is lost. Some of the compounds which have an acid reaction such as catechol and pyrogallol have a tendency to dissolve compounds of iron from storage tanks and these compounds have a dark color, dark blue or black, which tends to discolor the gasoline. These colored compounds are soluble in water and insoluble in gasoline but nevertheless the retailers of gasoline object to the presence of colored water solutions in the gasoline.

In accordance with the present invention it has been discovered that the poly-hydroxy-benzenes, particularly the poly-hydroxy-benzenes such as pyrogallol, catechol, and phloroglucinol, may be modified by attaching to the benzene nucleus hydrocarbon radicals which make the resulting compound substantially insoluble in water. Such compounds preserve the original grouping of the hydroxyl radicals on the benzene nucleus, thus preserving the gum-inhibiting or reducing properties of the compounds. Furthermore it has been found that straight chain hydrocarbons may be attached to the benzene nucleus as a modifying agent and this straight chain hydrocarbon can in turn be modified by attaching thereto side chain alkyl groups or amino groups to make the resulting compound gasoline-soluble, as well as being water-insoluble.

It further has been discovered that the hydrogen of one of the hydroxyl radicals of a tri-hydroxy-benzene may be substituted by an alkyl or straight chain hydrocarbon to form an ether which is substantially insoluble in water and this straight-chain hydrocarbon or alkyl group may be modified so as to make the compound gasoline-soluble as well as water-insoluble. In making ethers, however, it has been found that the best results are obtained when modifying only one hydroxyl so that the resulting compound retains two hydroxyl groups in the molecule.

Among the compounds which have been found to be particularly effective as gasoline stabilizers

are decyl-pyrogallol, hevyl-pyrogallol, alpha-ethyl-hexyl-pyrogallol, pyrogallol-mono-heptyl-ether, nonyl-pyrogallol and ethyl-octyl-pyrogallol. In general the compounds which have been found to be most satisfactory may be represented structurally as follows:



25 R is a straight chain hydrocarbon or a straight chain hydrocarbon modified with a side chain alkyl or amino group.



35 R' is an alkyl radical having C<sub>5</sub> or higher carbon atoms which may or may not be modified with a side chain amino or an alkyl group.

The modified straight chain hydrocarbons which may be attached to the benzene nucleus are straight chain hydrocarbons which have five 40 or more carbon atoms in the radical. It has been found that the alkyl groups having less than five carbon atoms do not generally form compounds which are insoluble in water as the straight chain hydrocarbon radicals which have five carbon atoms or more. Those compounds furthermore which are gasoline-soluble preferably have the straight chain hydrocarbon radical modified by a side chain alkyl or an amino group. The ether is preferably made by substituting a 45 straight chain hydrocarbon for a hydrogen of a hydroxyl group and this straight chain hydrocarbon may in turn be modified in order to render the compound soluble in gasoline.

To stabilize gasoline with the compounds mentioned above it is usually best to dissolve a small amount of the inhibiting compound with the gasoline when it is freshly made, that is soon after the gasoline is removed from the stills. If the gasoline is allowed to stand for any considerable 55 period after it has been made there is a polymerization or some form of rearrangement of the compounds which increases the difficulty of stabilizing the gasoline. Furthermore the gasoline is so altered that the refining process ends 60 a loss of gasoline.

When freshly made gasoline is treated with gum-inhibiting compounds in accordance with the present invention the amount used varies from .01 to .1% by weight of the gasoline. I 70 have found, however, that an inhibitor used in the ratio of 8 to 15 milligrams to 100 cc. of gasoline gives the best results. If too much inhibitor is used the tendency to develop gum-forming compounds is often accelerated.

75 In the treatments of gasolines it has been found

that cracked gasolines, particularly, contain two commonly-known forms of gum, a potential gum and a fixed gum. The usual tests for determining the content of the gasoline are the copper dish test, which consists in slowly vaporizing gasoline in a copper dish, and the pressure bomb test or accelerated storage test. The copper dish test is quite interesting and indicative of the character of the gum in some forms of gasoline but the accelerated bomb test is relied upon more 10 on account of the fact that it gives an indication of gum formation in the gasoline during long storage duration.

Some examples of the use of gum inhibitors, in accordance with the present invention, are 15 cited below. These tests, however, are not comparative of the action of the different inhibitors because the inhibitors have been used on different forms of gasoline, and gasolines having different 20 gum contents. Examples:

#### Alpha-ethyl-hexyl pyrogallol

|                                                    | Copper-dish<br>gum mgs.<br>per 100 cc. | Potential<br>gum mgs.<br>per 100 cc. | Pressure<br>drop in<br>bomb | 25     |
|----------------------------------------------------|----------------------------------------|--------------------------------------|-----------------------------|--------|
| Gasoline blank.....                                | 133                                    | .....                                | .....                       | Pounds |
| Gasoline+20 mgs. alpha-ethyl-hexyl pyrogallol..... | 90                                     | .....                                | .....                       | 30     |
| Gasoline blank.....                                | 1864                                   | .....                                | 40                          |        |
| Gasoline+30 mgs. alpha-ethyl-hexyl pyrogallol..... | 170                                    | .....                                | 2                           |        |

#### Decyl pyrogallol

|                                                                              |       |       |                        |    |
|------------------------------------------------------------------------------|-------|-------|------------------------|----|
| Gasoline blank.....                                                          | 11.00 | 1000  | .....                  | 35 |
| Gasoline+10 mgs. decyl pyrogallol.....                                       | 11    | 4     | .....                  |    |
| Gasoline+10 mgs. decyl pyrogallol washed with water.....                     | 11    | 4     | .....                  |    |
| Gasoline+10 mgs. decyl pyrogallol.....                                       | 5     | ..... | .....                  |    |
| Gasoline blank.....                                                          | 100   | 915   | 41                     | 40 |
| Gasoline+10 mgs. decyl pyrogallol.....                                       | 7     | 0     | None after<br>3 hours. |    |
| Gasoline+10 mgs. decyl pyrogallol washed 30 minutes<br>with turbo mixer..... | 8     | 0     | None.                  | 45 |

#### Decyl pyrogallol+anthracene

|                                                          |     |       |       |    |
|----------------------------------------------------------|-----|-------|-------|----|
| Gasoline blank.....                                      | 249 | ..... | ..... | 50 |
| Gasoline+10 mgs. decyl pyrogallol.....                   | 11  | ..... | ..... |    |
| Gasoline+10 mgs. decyl pyrogallol+2 mgs. anthracene..... | 3   | ..... | ..... |    |

#### Hexyl pyrogallol

|                                        |    |       |       |    |
|----------------------------------------|----|-------|-------|----|
| Gasoline blank.....                    | 39 | ..... | ..... | 55 |
| Gasoline+10 mgs. hexyl pyrogallol..... | 5  | ..... | ..... |    |

#### Ethyl octyl pyrogallol

|                                              |     |      |       |    |
|----------------------------------------------|-----|------|-------|----|
| Gasoline blank.....                          | 427 | 1506 | ..... | 60 |
| Gasoline+10 mgs. ethyl octyl pyrogallol..... | 11  | 22   | 0     |    |

In some cases where it is important to allow gasoline to stand in the light or sunlight it is 65 quite important to have the gasoline light-stable. Anthracene has the property of assisting in giving a light-stable gasoline and the properties are additive to the inhibitors of the present invention in giving a light-stable as well as a gum 70 and octane-stable gasoline. The amount of anthracene used with the preferred inhibitor is approximately the same as the amount of the preferred inhibitor.

The solubility of preferred inhibitors in gaso- 75

line need not be high provided that the inhibitor is more soluble in gasoline than in water. It is very desirable that all of the inhibitor be dissolved in the gasoline, otherwise some inhibitor 5 may stay in suspension or be precipitated and thus affect the color and quality of the gasoline. In order to readily dissolve the inhibitor in the gasoline it is desirable in many cases to dissolve the preferred inhibitor in dry alcohols or benzol 10 and then put the alcohol or benzol solution into the gasoline. It has been found that when the poly-hydroxy compounds have been modified with straight chain or modified straight chain hydrocarbons the products formed are very soluble 15 in most alcohols and benzol. One of the best solvents which has been used is a dry secondary butyl alcohol because this product is readily soluble in gasolines. It has also been found that the secondary amyl and hexyl alcohols when dry 20 are good solvents for the preferred inhibitors and are effective in dissolving the inhibitor in the gasoline. It has been found, furthermore, that the higher alcohols are not as readily soluble in water as the lower alcohols and therefore the 25 solution of these compounds in gasoline assists in preventing the inhibitor from being extracted from the gasoline when the gasoline is washed or contacted with water.

In the claims the term "gasoline" has been used 30 in defining the motor fuel, it being understood that gasoline is a distillate which may be obtained from any form of petroleum oil or coal tar oil.

Having thus described the invention, what is claimed is:

35 1. A motor fuel comprising cracked gasoline normally tending to develop gum on storage and a small amount of polyhydroxy benzene having an alkyl radical containing from 8 to 10 carbon atoms attached to a carbon atom of the benzene

nucleus, said alkylated polyhydroxy benzene being used in quantities sufficient to retard gum formation in the motor fuel.

2. A motor fuel comprising cracked gasoline 5 normally tending to develop gum on storage and having incorporated therein, in an amount sufficient to retard said gum formation, catechol having an alkyl radical containing from 8 to 10 carbon atoms attached directly to the benzene 10 nucleus of the catechol.

3. A motor fuel comprising cracked gasoline normally tending to deteriorate and develop gums on storage and having incorporated therein, in an amount sufficient to retard said gum formation, pyrogallol having an alkyl radical containing from 8 to 10 carbon atoms attached directly 15 to the benzene nucleus of the pyrogallol.

4. A motor fuel comprising cracked gasoline normally tending to deteriorate and develop gum on storage and having incorporated therein a 20 decyl pyrogallol in quantity sufficient to retard said gum formation.

5. A motor fuel comprising cracked gasoline normally tending to deteriorate and develop gum on storage and having incorporated therein al- 25 pha-ethyl-hexyl-pyrogallol in quantity sufficient to retard said gum formation.

6. A motor fuel comprising cracked gasoline normally tending to deteriorate and develop gum on storage and having incorporated therein 30 ethyl-octyl-pyrogallol in quantity sufficient to retard said gum formation.

7. A motor fuel comprising cracked gasoline normally tending to deteriorate and develop gum on storage and having incorporated therein an 35 octyl pyrogallol in quantity sufficient to retard said gum formation.

EDMUND G. BORDEN.